

# UNITED STATES PATENT OFFICE.

MAX LUFT, OF BORAS, SWEDEN.

## MANUFACTURE OF ARTIFICIAL GOODS FROM VISCOSE.

1,407,696.

Specification of Letters Patent. Patented Feb. 28, 1922.

No Drawing.

Application filed March 9, 1920. Serial No. 364,542.

To all whom it may concern:

Be it known that I, Dr. MAX LUFT, a citizen of Poland, residing at Boras, in Sweden, have invented certain new and use-

5 ful Improvements in Manufacture of Artificial Goods from Viscose; and I do hereby declare the following to be a full, clear, and exact description of the invention, such as will enable others skilled in the art to which

10 it appertains to make and use the same.

My invention relates to the manufacture of artificial fabrics, filaments, films and the like articles from viscose (cellulose-xanthate) and has for its object to render the 15 manufacture more expeditious and produce a cellulose which is of uniform character, consistency, lustre, and feel.

The manufacture of filaments, films, plates and the like from viscose, which forms an 20 unstable solution, depends upon several conditions, as for instance upon the state of maturation of the viscose, upon the several by-products and the partly gaseous objectionable products of decomposition of the xanthate. These conditions are practically for 25 the most part not controllable and cause great losses of material and affect the lustre, the strength, and the uniformity of the formed cellulose-hydrates.

30 I have found that the acids of the naphthalenes or the aqueous solutions of their salts added to the solution of xanthate have a surprisingly favorable effect, as they bind the sulphur-by-products and the impurities 35 of the viscose, improve the uniformity and durability of the solution and render the precipitation or separation of the cellulose-hydrates uniform and independent from the state of maturation of the raw viscose used.

40 The raw viscose treated with acids of the naphthalenes gives by the precipitation in acids or salt-solutions goods of an improved quality.

The acids of the naphthalenes (the carboxyl-derivatives of the naphthalenes or the polymethylenes) are to be found in large 45 quantities in petroleum (naphtha) and are obtained as waste-products from the distillation of petroleum in the form of alkaline 50 salts of the naphthalenes. Their affinity for sulphur and for sulphides is—according to

Renouard "Les matières grasses" 1919—so intensive that they are capable to devulcanize the caoutchouc and may be used for the regeneration of the same.

55

I found that in the alkaline solutions of viscose the acids of the naphthalenes bind the sulphides, thiocarbonates, and other impurities containing sulphur, without influencing in any way the xanthate. The viscose does not coagulate and the solutions remain 60 homogeneous. They may be used without further treatment for the manufacture of the artificial goods, for instance they may be spun in acid solutions of salts. The acid 65 of the naphthalenes freed from the threads during the spinning process continues to act in the spinning bath and hinders the adverse reactions of the sulphides taking place under ordinary circumstances. The 70 resulting products are smooth and uniform in lustre and softness as well as in strength and elasticity.

To carry out my process the liquid acid of 75 naphthalenes which ought to be free from resin or preferably the aqueous or alkaline solutions of the salt of the acid, is allowed to flow in and is uniformly mixed with the common alkaline solution of the xanthate. The waste solutions of the petroleum factories represents such an alkaline solution. The acid of naphthalenes or its salts may be 80 added to the finished solution of the viscose or to the alkaline water with which the viscose is stirred and diluted.

85 The quantity of the free acid of naphthalenes used depends upon the quantity of CS<sub>2</sub> required for the formation of the xanthate and is about five per cent of the latter quantity. The acids of the naphthalenes and 90 their sulphur compounds may be separated from the baths in the usual manner, recovered and used again, which renders the process much cheaper. The resulting artificial goods are thereupon washed and 95 treated in the common way.

I claim:

1. The improvement in the manufacture of 100 artificial goods from viscose consisting in the addition of acids of naphthalenes to the solution of viscose for the purpose described.

2. The improvement in the manufacture of

artificial goods from viscose consisting in the addition of acids of naphthenes together with alkaline diluting water to the xanthate as and for the purpose specified.

5. 3. The improvement in the manufacture of artificial goods from viscose consisting in

the addition to the viscose of any of the salts of the acids of naphthenes which are soluble in water as and for the purpose specified.

In testimony whereof I affix my signature.

MAX LUFT.

10